

## UNITED STATES PATENT OFFICE

HENRY DREYFUS, OF LONDON, ENGLAND

## TREATMENT OF CELLULOSE PRIOR TO ESTERIFICATION

No Drawing. Original application filed April 18, 1923, Serial No. 633,016, and in Great Britain May 24, 1922. Divided and this application filed July 23, 1927. Serial No. 209,191.

This application is a division of my prior application Serial No. 633,016 filed April 18, 1923 which eventuated into Patent 1,708,787 issued April 9, 1929.

The above application covers esterifying cellulose or its near conversion products with acetic or other fatty acid anhydride in presence of sulphuric acid or other strong condensing agent to produce a highly viscous product by means of using acetic acid or other solvent in quantity over 6 times the weight of the cellulose.

The subject matter of the present application relates to a preliminary treatment which may be given the cellulose or cellulose conversion products in order to render them more reactive to the esterification process while substantially preserving the strength of the cellulosic material. While cellulose or its conversion products which have been pretreated according to the process hereinafter described and claimed are especially suitable for esterification according to the process disclosed and claimed in said parent application, nevertheless they may be esterified by other known or new processes of esterification.

To carry out the invention one can treat the cellulose such as cotton or conversion product of cellulose with formic acid alone, either with heating or at ordinary temperature, or with cooling, but preferably at ordinary temperature or slightly higher.

Such a special pretreatment may also be carried out by treating the cellulose or cellulose conversion product by heating or boiling with concentrated or dilute formic acid, preferably with the addition of small quantities of sodium acetate or other suitable neutralizing agent which is capable of neutralizing any traces of mineral acids that may be present, and which mineral acid would have a destructive effect upon the cellulose molecules, especially during the hot treatment with formic acid. The cellulosic material may be treated either in the cold or hot with concentrated or dilute formic acid, preferably but not necessarily containing a small quantity of sodium acetate or other suitable neutralizing agent. The temperature and the

length of the treatment will vary with the concentration of the acid and also with the particular acid used.

In another divisional application S. No. 81,838 filed January 16, 1926, I have explained that cellulose may be pretreated for instance, with glacial acetic acid, at about 100° C. or at the boiling point of the acid, the treatment lasting about one to six hours, more or less, and being correspondingly longer at temperatures between about 80° and 100° C. Similarly, with more dilute acid, such as acetic acid of from 80% to 50% strength or less, the hot treatment will take correspondingly longer for a given temperature dependent upon the increased dilution of the acid.

When formic acid is used, however, although it may be employed in a concentrated form, this is less advantageous and it is better to use a more dilute acid of about 50% strength or upwards. This will effect the pretreatment more quickly even than a more concentrated acetic acid, and especially it is in this case advantageous to employ it in the cold. When a more dilute acid is used, a hot treatment is preferably adopted.

In any of the forms of pretreatment above described, the formic acid employed may be used in admixture with diluents which are not capable of entering into reaction with either the cellulose or the acid, such as toluol. This is found to be somewhat less advantageous.

The pretreated material may be subjected directly to the esterifying reaction, but it is found preferable to wash and dry the same before subjecting it to esterification.

When cellulose or its conversion products are thus pretreated, the esterification process is carried out more quickly, and it is possible, when using sulphuric acid or other strong condensing agent, to conduct and finish acetylation at temperatures as low as 0° C. or even lower. Of course since the esterification reaction with such pretreated material is much more effective, higher temperatures may be employed by using increased quantities of acetic acid or diluent in the esterification process. Thus, the esterification may be per-

formed at ordinary temperature or even at higher temperatures. Of course, with weak or very weak condensing agents, proportionately higher temperatures are necessary.

5 Although of particular value in the production of cellulose acetate, the pretreatment which forms the subject matter of the present invention is of value in the production of any of the fatty acid esters of cellulose. The 10 invention is, therefore, to be regarded as limited only by the scope of the appended claims.

What I claim and desire to secure by Letters Patent is:—

15 1. A process for pretreating cellulose, which comprises subjecting it to the action of formic acid in the absence of a condensing agent, thereby rendering the cellulose capable of rapid esterification.

20 2. A process for pretreating cellulose, which comprises subjecting it to the action of formic acid of not less than 50% concentration in the absence of a condensing agent, thereby rendering the cellulose capable of rapid esterification.

25 3. A process for treating cellulose, which comprises pretreating it with formic acid to render the cellulose capable of rapid esterification, and afterwards subjecting it to the action of an esterifying medium.

30 4. A process for treating cellulose, which comprises pretreating it with formic acid to render the cellulose capable of rapid esterification, removing the formic acid from the cellulose, and afterwards subjecting the cellulose to the action of an esterifying medium.

35 5. A process for treating cellulose, which comprises pretreating it with formic acid to render the cellulose capable of rapid esterification, and afterwards subjecting it to the action of an acetylating medium.

40 6. A process for treating cellulose, which comprises pretreating it with formic acid to render the cellulose capable of rapid esterification, removing the formic acid from the cellulose, and afterwards subjecting the cellulose to the action of an acetylating medium.

45 7. A process for pretreating cellulose, which comprises subjecting it to the action of formic acid in the absence of a condensing agent and in the presence of a diluent inert to the cellulose and the acid, thereby rendering the cellulose capable of rapid esterification.

50 8. A process for pretreating cellulose, which comprises subjecting it to the action of formic acid containing a small quantity of a neutralizing agent for mineral acid, thereby rendering the cellulose capable of rapid esterification.

55 9. A process for pretreating cellulose, which comprises subjecting it to the action of formic acid containing a small quantity of sodium acetate, thereby rendering the cellulose capable of rapid esterification.

10. A process for pretreating cellulose, which comprises subjecting it to the action of formic acid of not less than 50% concentration and containing a small quantity of sodium acetate, thereby rendering the cellulose capable of rapid esterification. 70

11. A process for pretreating cellulose, which comprises subjecting it to the action of concentrated formic acid in the substantial absence of a condensing agent, thereby rendering the cellulose capable of rapid esterification. 75

12. A process for treating cellulose, which comprises pretreating it with a concentrated formic acid to render the cellulose capable of rapid esterification, and afterwards subjecting it to the action of an esterifying medium. 80

13. A process for treating cellulose, which comprises pretreating it with a concentrated formic acid to render the cellulose capable of rapid esterification, and afterwards subjecting it to the action of an acetylating medium. 85

In testimony whereof I have hereunto subscribed my name.

HENRY DREYFUS.

95

100

105

110

115

120

125

130